

# UNITED STATES PATENT OFFICE.

GEORGE M. MOWBRAY, OF ADAMS, MASSACHUSETTS, ASSIGNOR TO THE AMERICAN ZYLONITE COMPANY, OF SAME PLACE.

## PLASTIC COMPOUND RESEMBLING IVORY.

SPECIFICATION forming part of Letters Patent No. 320,884, dated June 23, 1885.

Application filed February 16, 1884. (Specimens.)

*To all whom it may concern:*

Be it known that I, GEORGE M. MOWBRAY, a citizen of the United States, residing at Adams, in the county of Berkshire and State of Massachusetts, have invented new and useful Improvements in Plastic Compounds, of which the following is a specification.

The nature of my invention consists in a certain composition of matter and in the method of blending its components so as to produce a very close imitation of ivory, wherein I use soluble pyroxyline as the counterpart of the gelatine, and finely-divided neutral matter—such as precipitated sulphate barytes, silicate of alumina, &c.—as the counterpart of the skeleton frame of the natural tusk.

Various materials have been used to imitate this valuable material, among others, in a patent granted to J. B. Edson, No. 283,225, August 14, 1883, a composition of pyroxyline and inert matters is described, where the different growths or layers of zylonite are either of differing densities or different colors, so as to indicate the grain of the natural tusk by these characteristics.

Now, my invention secures a homogeneous compound of like density throughout, the surface only of the rolled sheets being tinted with a slight stain of color, the result being a closer imitation of natural ivory, the manipulation more facile, and with the ingredients used as hereinafter described a translucency peculiar to natural ivory is obtained.

The ingredients I prefer and their proportions are: of soluble pyroxyline, about ten parts; of camphor, from four to five parts; of precipitated sulphate barytes, about three parts; oxide of zinc, either precipitated or sublimed, one part. Better results are obtained by reducing these ingredients to a fine state of division, rendering them perfectly dry, and thoroughly mixing together, and then adding either of the following solvents or a mixture of any of them, viz: ethylic alcohol, methylic alcohol, or methylated spirits, say, about six parts, the solvent being added to the mixture of pyroxyline and neutral matters mentioned above. The agglutinated mass is subjected to heat and pressure effected between a pair of rolls in the usual man-

ner well known in the art, so as to reduce the material into sheets, the thickness of which may vary from about one thirty-second to one-sixteenth of an inch. Alternate sheets are then dipped either into a very dilute solution of aniline-yellow of a tint that will imitate the grain of the natural tusk, or the surface of each sheet or of each alternate sheet is then painted over with a very dilute wash of aniline-yellow, one part of the aniline to one thousand and parts of alcohol being ample. The sheets are now bundled up in layers and submitted to pressure until a perfect weld of each layer to the next is effected. These sheets thus welded together are then ready for manufacturing purposes, and can be reduced to such forms as may be required by any method known to the art.

I do not confine myself to the exact proportions of the ingredients above specified, since the proportions may be varied somewhat without injuring the product; nor am I to be confined to the neutral matter or metallic oxide specified above, there being many neutral materials and other oxides that serve as equivalents for those specified; but the above ingredients in the proportions specified and combined in the manner directed have yielded me a composition of matter very closely resembling the natural ivory tusk.

Having thus described my invention, what I claim is—

1. The within process of producing imitation ivory, consisting in tinting the surface of layers of a composition of pyroxyline and inert matters with coloring-matter, substantially as described.

2. The within process of producing imitation ivory, consisting in coloring the surface of the layers or alternate layers of pyroxyline compound and then uniting the same to other layers of like composition, substantially as set forth.

3. The within process of producing imitation ivory, consisting in forming a composition of pyroxyline and neutral matters, then sheeting the same, next coloring the surfaces of sheets of such composition and uniting such sheets together by pressure, substantially as described.

4. As a new article of manufacture, a pro-

duct composed of a series of sheets of a composition of pyroxylene and neutral matter of uniform composition, with at least one surface of the superposed sheets colored and the sections united together either by heat and pressure or by solvents and pressure, substantially as described.

In testimony whereof I have hereunto set my hand and seal in the presence of two subscribing witnesses.

GEO. M. MOWBRAY. [L. S.]  
Witnesses:

RUSL. B. DEAN,  
S. W. INGALLS.